

1

3,781,204

### TEXTILE TREATING COMPOSITION

Mamoru Katsumi, Toshio Sato, and Tadao Hara, Wakayama, Japan, assignors to Kao Soap Co., Ltd., Tokyo, Japan

No Drawing. Filed Dec. 17, 1971, Ser. No. 209,454  
Claims priority, application Japan, Dec. 23, 1970,  
45/117,164

Int. Cl. D06m 13/46; B44d 5/06  
U.S. Cl. 252—8.75

1 Claim

### ABSTRACT OF THE DISCLOSURE

A textile treating composition essentially consisting of the following three ingredients (1) to (3):

(1) 1 to 10 parts by weight of a cationic surface active agent of the general formula:



wherein  $R_1$  and  $R_2$  are alkyl radicals of 12-22 carbon atoms,  $R_3$  and  $R_4$  are alkyl radicals of 1-4 carbon atoms and  $X^-$  is a halogen ion,  $CH_3SO_4^-$  or

$C_2H_5SO_4^-$ ,

(2) 0.05 to 0.5 part by weight of an optical brightener of the general formula:



wherein  $M$  is an alkali metal or an ethanol amine, and

(3) 0.5 to 10 parts by weight of a cationic surface active agent which is characterized by that

(i) it has one or more of cationic nitrogen atoms in a molecule,

(ii) it has 1 to 3 polyoxyethylene groups attached on said cationic nitrogen atoms, each of the polyoxyethylene groups having a terminal hydroxy radical and having oxyethylene units of 1-14 moles, and

(iii) it has one or two of  $RCH_2^-$ ,  $RCONH(CH_2)_n^-$  or  $RCOO(CH_2)_n^-$ , in which  $R$  is an alkyl radical of 11-21 carbon atoms and  $n$  is an integer of 1 to 3, in a molecule.

The present invention relates to a textile treating composition. More particularly, the present invention relates to a fabric softener having optical brighteners incorporated therewith.

Domestic fabric softeners have excellent effects such as softening of textile for providing nice feeling, preventing the accumulation of electrostatic charge on synthetic textile, conditioning textile for smooth ironing and shortening the drying time. Main ingredients of domestic fabric softeners are generally cationic surface active agents of the following general Formula I:



(I)

wherein  $R_1$  and  $R_2$  represent alkyl radicals of 12-22 carbon atoms,  $R_3$  and  $R_4$  represent alkyl radicals of 1-4 carbon atoms, and  $X^-$  represents a halogen ion,  $C_2H_5SO_4^-$  or  $CH_3SO_4^-$ .

Although domestic fabric softeners have such various excellent effects as mentioned above, they have a dis-

2

advantage that, when they are applied to commercial textiles which are finished with an anionic optical brightener, the textiles are often yellowed, because the anionic optical brightener reacts with the cationic softening agent and then fluorescence is quenched. In order to prevent the textiles from yellowing, optical brighteners are usually added to softening agents. However, when any of usual softening agents is employed, the quantity of the optical brightener adsorbed on the textile is rather small so that a sufficient whitening effect is never expected.

Some studies have been published which were made for the purpose of overcoming these defects, which are as follows:

(A) Optical brighteners of bis-(triazinylamino)stilbene-disulfonicacid having the following general Formula II, which is compatible with said cationic surface active agent represented by the above general Formula I have been described in "Optical Brighteners in Fabric Softeners" [Soap & Chemical Specialities, 40, 85-88 (May in 1965)].



wherein  $X$  is



30 Y is



35 and  $M$  represents Na, K or an ethanolamine.

When these optical brighteners are employed, the compositions have to satisfy the following two requirements, that is;

- 40 (a) They must contain no inorganic electrolyte.  
(b) The solubility of the complex salt of the cationic surface active agent and the optical brightener in water should be large.

45 However, in order to satisfy the above requirement (b), 50 X of the optical brightener represented by the above general Formula II should be



55 and  $Y$  should be a radical of the structure having remarkably hydrophilic hydroxyethyl groups, and when such a requirement is chosen, the composition is surely stable. However, as described in the papers and shown in the hereinafter described examples, when this composition is employed for the treatment of textiles, the adsorbed optical brightener is scarcely detected, and, therefore, it cannot be employed practically. It is impossible to prevent the quenching of fluorescence on textiles which is caused by a cationic surface active agent, and to bring about an improvement of the substantivity of optical brighteners incorporated in a fabric softener.

60 (B) Since a cationic surface active agent such as the compounds as shown by the Formula I is used as a fabric softener, it is expected that, if a cationic optical brightener is added to a fabric brightener, the substantivity of the optical brightener might be improved. As such cationic

optical brightener, there are, for example, Tinopal AN of the oxycyanine type (produced by J. R. Geigy, Switzerland, which has the following Formula III;



wherein R is a lower alkyl radical, X⁻ is an anion such as a halogen ion, etc., and Daitophor AN of the bis-oxazol types (produced by Daito Chemical Co., Japan, which has the following Formula IV;



In principle, these agents have to show a sufficient whitening effect in a fabric softener, but they have, in fact, an excellent whitening effect only as to poly-acrylonitrile textiles and they do not show a sufficient substantivity to other textiles. Accordingly, they are not desirable optical brighteners in case these agents should be incorporated into the softening agents for underwears, diaper and sweater, etc., which are made of cellulose fibers. Further, most optical brighteners, which are to be blended in detergents and to be used for whitening cellulose textiles, are of anionic stilbene type, so that these anionic optical brighteners react with the aforesaid cationic optical brighteners in a treating bath to form a complex which will cause to decrease the effect of preventing yellowing and the whitening effect. This will be distinctly observed in treating a textile, which has been finished with an anionic optical brightener, by a cycle which is arranged in the order of washing → softening → drying → washing → . . . . Consequently, it cannot be said that the effects of preventing the yellowing and whitening of textiles by treating textiles with a fabric softener, mixed with a known optical brightener, are satisfactory.

We have studied about the effective prevention of yellowing and the effective whitening of the textile by the use of a fabric softener of which the main ingredient is a cationic surface active agent of the above general Formula I and could attain the purpose by the following novel textile treating compositions.

The composition of the present invention consists essentially of the following three ingredients.

They are a cationic surface active agent of the above general Formula I (first ingredient), sodium distilbene-disulfonate of the following Formula V (second ingredient);



wherein M represents an alkali metal such as Na or K, or an ethanolamine, and a cationic surface active agent (third ingredient), which is characterized by the facts that (1) it has one or more of cationic nitrogen atoms in a molecule, (2) it has 1 to 3 polyoxyethylene groups attached on said cationic nitrogen atoms, each polyoxyethylene group having a terminal hydroxy radical and 75

having oxyethylene units of 1-14 moles and (3) it has one or two of



5 (wherein R is an alkyl radical of 11-21 carbon atoms and n is an integer of 1 to 3) in a molecule.

The fabric softener composition consisting essentially of the above three ingredients according to the present invention is excellent in the prevention of yellowing and the whitening of textiles. This composition doesn't react with any of stilbene-type optical brighteners which have been often used for commercially available clothes, so that the yellowing of textiles does not substantially happen. Moreover, the substantivity of the above second in-

10 gredient to textiles is better than any known optical brightener. However, in case the fabric softener composition consists only of the first and second ingredients, not containing the third ingredient, the aforesaid effects would not be obtained. In other words, the effect of preventing

15 the yellowing and increasing the whitening effects would not be substantially obtained. The same can be said of a fabric softener composition consisting only of the first and third ingredients, and not containing the second ingredient.

20 25 That is to say, the composition of the present invention is not significantly characterized by either one of the second ingredient and the third ingredient, but rather requires the combination of the above first, second and third ingredients. The respective ingredient cannot be

30 35 replaced by other similar compounds. Effective prevention of yellowing and effective whitening can be obtained only by this combination of the above three ingredients.

In addition, the third ingredient can prevent the "Tinting 40 45 phenomenon" of the optical brightener. (The "Tinting phenomenon" is a phenomenon that the optical brightener is put in spots on textiles.) Therefore, the composition shows a uniform whitening effect on textile fabrics. Furthermore, the third ingredient reduces the solution viscosity of the fabric softener so that it can be smoothly

40 45 poured and prevents precipitation after a long storage.

A theoretical explanation of the effects to be obtained by the ternary system of the present invention, which are the prevention of yellowing, the improvement of whitening and the prevention of tinting phenomenon, is not yet

50 55 possible, but it is presumed to be as follows:

The above cationic surface active agent of the general Formula I and the above optical brightener of the general Formula V are reacted in an aqueous solution to form a complex which tends to be precipitated. However, when a compound having polyoxyethylene groups in the molecule such as the above third ingredient co-exists, the complex may stay stably in the solution and the physico-chemical affinity of the complex mainly to cellulosic textiles may be promoted. To this end, it is required that the oxyethylene units in the polyoxyethylene group is about 1 to 14 moles. In case this is more than 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255

$-\text{CH}_2\text{R}_{15}$ ,  $-(\text{CH}_2)_k\text{NHCOR}_{15}$  or  $-(\text{CH}_2)_k\text{OOCR}_{15}$  (wherein  $\text{R}_{15}$  is an alkyl radical of 11-21 carbon atoms,  $k$  is an integer of from 1 to 3), and either one of  $\text{R}_{11}$  and  $\text{R}_{12}$  is  $-\text{CH}_2\text{R}_{15}$ ,  $-(\text{CH}_2)_k\text{NHCOR}_{15}$  or



$\text{R}_{13}$  represents  $-\text{CH}_3$ ,  $-\text{C}_2\text{H}_5$ ,



or  $-(\text{CH}_2\text{CH}_2\text{O})_m\text{H}$ ,  $\text{R}_{14}$  represents  $-(\text{CH}_2\text{CH}_2)_n\text{H}$ ,  $m$  and  $n$  each represent an integer of more than 1, and  $2 \leq m+n \leq 14$ ,  $\text{X}_1^-$  represents a halogen ion,  $\text{CH}_3\text{SO}_4^-$  or  $\text{C}_2\text{H}_5\text{SO}_4^-$ .



wherein  $\text{R}_{21}$  represents  $-\text{CH}_2\text{R}_{26}$ ,  $-(\text{CH}_2)_k\text{NHCOR}_{26}$  or  $-(\text{CH}_2)_k\text{OOCCH}_{26}$  (wherein  $\text{R}_{26}$  is an alkyl radical of 11-21 carbon atoms,  $k$  is an integer of from 1 to 3),  $\text{R}_{22}$ ,  $\text{R}_{23}$  and  $\text{R}_{24}$  represent  $-(\text{CH}_2\text{CH}_2\text{O})_l\text{H}$ ,



or  $-(\text{CH}_2\text{CH}_2\text{O})_n\text{H}$  respectively,  $l$ ,  $m$  and  $n$  represent an integer of more than 1 and  $3 \leq l+m+n \leq 14$ , respectively.  $\text{R}_{25}$  represents  $-\text{CH}_3$ ,  $-\text{C}_2\text{H}_5$  or



$\text{X}_2^-$ ,  $\text{Y}_2^-$  represent a halogen ion,  $\text{CH}_3\text{SO}_4^-$  or  $\text{C}_2\text{H}_5\text{SO}_4^-$ , and  $i$  represents an integer of from 2 to 3.



wherein  $\text{R}_{31}$  and  $\text{R}_{32}$  represent alkyl radicals of 12-21 carbon atoms,  $\text{R}_{33}$  represents an alkylene radical of more than 2 carbon atoms,  $\text{R}_{34}$  represents  $-\text{CH}_3$ ,  $-\text{C}_2\text{H}_5$  or



$m$  and  $n$  represent an integer of more than 1 and

$$2 \leq m+n \leq 14$$

respectively,  $x$  and  $y$  each represent an integer of more than 1 and  $2 \leq x+y \leq 14$ , respectively,  $\text{X}_3^-$ ,  $\text{Y}_3^-$  represent a halogen ion,  $\text{CH}_3\text{SO}_4^-$  or  $\text{C}_2\text{H}_5\text{SO}_4^-$ .



wherein  $\text{M}$  represents



$\text{R}_{40}$  is an alkyl radical of 12-21 carbon atoms,  $s$  is 2 or 3,  $p$ ,  $q$  are an integer of more than 1 and  $2 \leq p+q \leq 14$ , respectively,  $\text{X}_4^-$  is an anion which will be derived from acetic acid, lactic acid, hydroxyacetic acid, boric acid or benzoic acid by removing one hydrogen from these acids.



wherein  $\text{R}_{50}$  is an alkyl radical of 11-21 carbon atoms,  $\text{X}_5^-$  is a halogen ion,  $\text{CH}_3\text{SO}_4^-$  or  $\text{C}_2\text{H}_5\text{SO}_4^-$ ,  $t$  is an integer from 1 to 14,  $\text{R}_{15}$  is  $-\text{CH}_3$ ,  $-\text{C}_2\text{H}_5$  or



wherein  $\text{R}_{50}$  is an alkyl radical of 11-21 carbon atoms.

As described above, the composition according to the present invention consists essentially of a combination of the above three ingredients and its unexpected remarkable effects could be obtained by the synergistic action of these ingredients.

The purpose of the present invention can be attained by blending said three ingredients in an appropriate blending ratio. It is preferable to blend these ingredients in the ratio that the first ingredient is 1 to 10 parts, the second ingredient is 0.05 to 0.5 part and the third ingredient is 0.5 to 10 parts respectively, in which all parts are parts by weight.

The present invention is further illustrated by the following examples.

#### EXAMPLE

The details of the three ingredients which were used in the following formulations according to the present invention are as follows:

##### Softening agent (first ingredient)

Percent by wt.

No. 1:  
Distearyl dimethyl ammonium chloride ----- 75  
Isopropylalcohol ----- 19  
Water ----- 6

No. 2:  
Dilauryl diethyl ammonium ethylsulfate ----- 75  
Isopropylalcohol ----- 19  
Water ----- 6

##### Optical brightener (second ingredient)

No. 1: An optical brightener having the above Formula II, in which



and which is commercially available under the trade name of Tinopal 2B (produced by J. R. Geigy). Its  $\lambda_{\text{max}}$  is 440 m $\mu$ .

No. 2: An optical brightener having the Formula II, in which



Its  $\lambda_{\text{max}}$  is 440 m $\mu$ .

No. 3: An optical brightener having the formula



which is commercially available under the trade name of Whitex R Extra Conc. (produced by Sumitomo Chemical Co.). Its  $\lambda_{\max}$  is 425 m $\mu$ .

No. 4: An optical brightener of the general Formula III, which is commercially available under the trade name of Tinopal AN (produced by J. R. Geigy). Its  $\lambda_{\max}$  is 420 m $\mu$ .

No. 5: An optical brightener of the general Formula IV, which is available under the trade name of Daitophor AN (produced by Daito Chemical Co.). Its  $\lambda_{\max}$  is 430 m $\mu$ .

No. 6: An optical brightener of the general Formula V. Its  $\lambda_{\max}$  is 435 m $\mu$ .

Before the use, optical brighteners were purified by precipitating crystals through acidification and reneutralizing the extracted crystals or by recrystallizing them from ethanol or acetone and then desalting the crystals.

### Third ingredient

No. 1: Stearyl-trimethylammonium chloride.

No. 2: Stearyl-di(polyethoxy)methylammonium chloride containing 2 moles of ethylene oxide.

No. 3: Lauryl-di(polyethoxy)ethylammonium ethylsulfate containing 10 moles of ethylene oxide.

No. 4: Myristyl-di(polyethoxy)methylammonium chloride containing 14 moles of ethylene oxide.

No. 5: Stearyl-di(polyethoxy)methylammonium chloride containing 20 moles of ethylene oxide.

No. 6: Stearyl-polyethoxymethylbenzylammonium chloride containing 8 moles of ethylene oxide.

No. 7: Stearyl-polyethoxymethylbenzylammonium chloride containing 20 moles of ethylene oxide.

No. 8: Dicoconutalkyl-polyethoxymethylammonium chloride containing 2 moles of ethylene oxide.

No. 9: N-stearyl-N,N'-diethyl-tri-(polyoxyethylene) ethylene-diammonium diethylsulfate containing 10 moles of ethylene oxide.

No. 10: N-lauryl-N,N'-dimethyl-tri-(polyoxyethylene) propylene-diammonium dichloride containing 3 moles of ethylene oxide.

No. 11: N-stearylaminoethyl-N,N-dimethyl-tri-(polyoxyethylene)ethylene-diammonium dichloride containing 12 moles of ethylene oxide.

No. 12: N-lauroyloxypropyl-N,N-diethyl-tri-(polyoxyethylene)-propylene-diammonium ethylsulfate containing 10 moles of ethylene oxide.

No. 13: N-lauryl-N,N'-dimethyl-tri-(polyoxyethylene) propylenediammonium dimethylsulfate containing 30 moles of ethylene oxide.

No. 14: A compound shown by the general Formula VIII, wherein R<sub>31</sub>, R<sub>32</sub> are alaryl radicals, R<sub>33</sub> is an adipic acid residue of 4 carbon atoms, R<sub>34</sub> is methyl, m+n=10, x+y=10 and X<sub>3</sub><sup>-</sup>, Y<sub>3</sub><sup>-</sup>=Cl<sup>-</sup>, Cl<sup>-</sup>.

No. 15: A compound which is same with the compound No. 14, except that m+n=20 and x+y=20.

No. 16: A salt of N,N'-distearoylaminoethyl-N,N'-di-hydroxyethylurea with acetic acid (the mole ratio is 1:1).

No. 17: N,N'-dilauroylaminoethyl-N,N'-di(polyoxyethylene)biuret lactate containing 10 moles of ethylene oxide.

No. 18: N,N'-dilauroylaminoethyleneaminoethylenurea acetate:



No. 19: 1-ethyl-1-hydroxyethyl-2-stearylimidazolinium ethylsulfate of the Formula X.

No. 20: Sodium 1-hydroxyethyl-1-carboxy-2-stearyl-imidazoliniumhydroxide of the Formula XI.

No. 21: 1-(acetylaminoethyl)-2-heptadecyl imidazolinium formate of the formula:



No. 22: Polyoxyethylene nonoylphenylether (P=10).

|                            | Parts by wt. |
|----------------------------|--------------|
| Softening agent No. 1      | 8            |
| Optical brightener No. 6   | 0.2          |
| The third ingredient No. 1 | 2            |
| Ethylene glycol            | 6            |
| NaCl                       | 0.05         |
| Water                      | Balance      |

20 The total amount is made to be 100 parts by weight in all formulations.

### Formulation 2:

As the third ingredient No. 2 was used and other materials were same as in Formulation 1.

|                            | Parts by wt. |
|----------------------------|--------------|
| Softening agent No. 1      | 9            |
| Optical brightener No. 6   | 0.2          |
| The third ingredient No. 3 | 1.5          |
| Ethylene glycol            | 6            |
| KCl                        | 0.02         |
| Water                      | Balance      |

### Formulation 4:

35 Except using No. 4 as the third ingredient, other materials were same as in Formulation 3.

### Formulation 5:

Except using No. 5 as the third ingredient, other materials were same as in Formulation 3.

### Formulation 6:

|                            | Parts by wt. |
|----------------------------|--------------|
| Softening agent No. 2      | 8.0          |
| Optical brightener No. 6   | 0.3          |
| The third ingredient No. 6 | 3            |
| Diethylene glycol          | 5            |
| NH <sub>4</sub> Cl         | 0.04         |
| Water                      | Balance      |

### Formulation 7:

50 Except using No. 7 as the third ingredient, other materials were the same as in Formulation 6.

### Formulation 8:

Except using No. 8 as the third ingredient, other materials were same as in Formulation 6.

### Formulation 9:

|                            | Parts by wt. |
|----------------------------|--------------|
| Softening agent No. 1      | 5            |
| Optical brightener No. 6   | 0.1          |
| The third ingredient No. 9 | 5            |
| Isopropylalcohol           | 5            |
| NaCl                       | 0.05         |
| Water                      | Balance      |

### Formulation 10:

65 Except using No. 10 as the third ingredient, other materials were same as in Formulation 9.

### Formulation 11:

Except using No. 11 as the third ingredient, other materials were same as in Formulation 9.

### Formulation 12:

70 Except using No. 12 as the third ingredient, other materials were same as in Formulation 9.

### Formulation 13:

Except using No. 13 as the third ingredient, other materials were same as in Formulation 9.

## Formulation 14:

|                             | Parts by wt. |
|-----------------------------|--------------|
| Softening agent No. 1       | 7            |
| Optical brightener No. 6    | 0.2          |
| The third ingredient No. 14 | 3            |
| Ethanol                     | 5            |
| Urea                        | 3            |
| NaCl                        | 0.05         |
| Water                       | Balance      |

## Formulation 15:

Except using No. 15 as the third ingredient, other materials were same as in Formulation 14.

## Formulation 16:

|                             | Parts by wt. |
|-----------------------------|--------------|
| Softening agent No. 1       | 6            |
| Optical brightener No. 6    | 0.4          |
| The third ingredient No. 16 | 4            |
| Propylene glycol            | 5            |
| NaCl                        | 0.02         |
| Water                       | Balance      |

## Formulation 17:

Except using No. 17 as the third ingredient, other materials were same as in Formulation 16.

## Formulation 18:

Except using No. 18 as the third ingredient, other materials were same as in Formulation 16.

## Formulation 19:

|                             | Parts by wt. |
|-----------------------------|--------------|
| Softening agent No. 2       | 5            |
| Optical brightener No. 6    | 0.2          |
| The third ingredient No. 19 | 5            |
| Ethylene glycol             | 2            |
| KCl                         | 0.05         |
| Water                       | Balance      |

## Formulation 20:

Except using No. 20 as the third ingredient, other materials were same as in Formulation 19.

## Formulation 21:

Except using No. 21 as the third ingredient, other materials were same as in Formulation 19.

## Formulation 22:

Except using No. 22 as the third ingredient, other materials were same as in Formulation 19.

## Formulation 23:

|                       | Parts by wt. |
|-----------------------|--------------|
| Softening agent No. 1 | 8            |
| Optical brightener    | 0.2          |
| The third ingredient  | None         |
| Ethylene glycol       | 6            |
| NaCl                  | 0.05         |
| Water                 | Balance      |

## Formulation 24:

Except using No. 1 as the optical brightener, other materials were same as in Formulation 1.

## Formulation 25:

Except using No. 3 as the optical brightener, other materials were same as in Formulation 1.

## Formulation 26:

Except using No. 2 as the optical brightener, other materials were same as in Formulation 6.

## Formulation 27:

Except using No. 4 as the optical brightener, other materials were same as in Formulation 1.

## Formulation 28:

Except using No. 5 as the optical brightener, other materials were same as in Formulation 6.

## Formulation 29:

|                             | Parts by wt. |
|-----------------------------|--------------|
| Softening agent No. 1       | 8            |
| Optical brightener No. 1    | 0.3          |
| The third ingredient No. 22 | 1.0          |
| Ethylene glycol             | 5            |
| NaCl                        | 0.05         |
| Water                       | Balance      |

## Formulation 30:

Except using No. 4 as the optical brightener, other materials were same as in Formulation 29.

With respect to the softener composition of the above formulations, the following tests were conducted.

## TEST 1

Judgments of effects concerning the prevention of yellowing the improvement of whitening and the tinting phenomenon

Bleached Cotton Broad #60 swatches (Reflectance: 89) and these broad swatches treated by a stilbene type optical brightener, Whitex BB conc. (produced by Sumitomo Chemical and Industrial Co.—commercial name— $\lambda_{\text{max.}}$ : 440 m $\mu$ ) were treated with said softener compositions (Formulations 1 to 30) under the following conditions.

Concentration of the softener composition, percent... 0.2  
The ratio of the swatch to the aqueous treating solution ..... 1:100  
Treating time ..... minutes... 5  
Temperature ..... °C... 30  
Sun-dried after removing water centrifugally.

As to the thus treated textiles the reflectance of each swatch was measured by the use of a spectrophotometer (Hitachi fluorophotoreflectometer FR-1 in the EPU-2A type spectrophotometer).

Reflectances of the swatches were measured at the maximum reflection wave  $\lambda_{\text{max.}}$  by using a filter of the effective wave width of 5.0 m $\mu$ . These reflectance data do not necessarily show a complete agreement with the naked eye observation.

Therefore, the whiteness was evaluated as the next criteria by 5 persons with their naked eyes under day light, and it was graded by the total of the points evaluated by 5 persons.

## Criteria of judgment

|                                             |    |
|---------------------------------------------|----|
| Sufficiently white in comparison with blank | +2 |
| Fairly white in comparison with blank       | +1 |
| No difference                               | 0  |
| Fairly less white than blank                | -1 |
| Remarkably less white than blank            | -2 |

The tinting phenomenon was evaluated by examining the treated swatches under ultraviolet light (black light), in which the following criteria were used.

## Criteria of judgment

|                                                              |    |
|--------------------------------------------------------------|----|
| No tinting, having the optical brightener uniformly adsorbed | +1 |
| Middle                                                       | +3 |
| Much tinting (Formulation No. 25 was presumed to be point 5) | +5 |

The results were shown in Table 1.

## TEST 2

## The effect of whitening by the repeated treatments

The swatches of Broad #60 (polyester-cotton (35-65) mixed, which was not treated with optical brightener, was washed with a commercial detergent (containing a stilbene-type optical brightener) and the swatches were treated with 0.1% aqueous solution of the above softening compositions in the 1/40 of swatches/solution weight ratio, and squeezed and air-dried. After the washing-softening-drying cycles were repeated 5 and 10 times, the whiteness (reflectance) was examined in the manner as described above.

The results were shown in Table 1.

**11**  
TEST 3

Stability of the formulations

After storing the aforesaid compositions at  $-5^{\circ}\text{C}$ ,  $20^{\circ}\text{C}$ , or  $40^{\circ}\text{C}$ . for two months, their stabilities were first examined with eye to check their phase separation or synergises, etc. and also they were checked under black light as to if they had troubles such as separation of optical brightener or its precipitation, etc.

The results were shown in Table 1.

5

**12**

than 15 will show excellent effects in the stabilization of the solution and in reducing the tinting phenomenon. The formulations 6, 7 and 8 relate to examples having one  $-(\text{CH}_2\text{CH}_2\text{O})_n\text{H}$  chain, and the formulation 8 relates to an example having two long chain alkyl radicals.

(2) The formulations 9 to 13 are examples having a compound of the general Formula VII. The formulations 9 to 12 relate to examples having



TABLE 1

Results in the Tests 1 to 3 as to prevention of yellowing, whitening effects, tinting phenomena and solution stability

| Formulation | Prevention effect of yellowing and whitening effect in Test 1 |                           |                                      | Judged value of tinting phenomena | Reflectance by Test 2 | Solution stability by Test 3                                    |
|-------------|---------------------------------------------------------------|---------------------------|--------------------------------------|-----------------------------------|-----------------------|-----------------------------------------------------------------|
|             | Swatches not finished with optical brightener                 |                           | Swatches finished optical brightener |                                   |                       |                                                                 |
|             | Reflectance                                                   | Judg-<br>ment with<br>eye | Reflectance                          | Judg-<br>ment with<br>eye         |                       |                                                                 |
| 1           | 92                                                            | 2                         | 120                                  | -3                                | 5                     | 118 Phase separation, precipitation of optical brighteners.     |
| 2           | 109                                                           | 9                         | 127                                  | 3                                 | 1                     | 131 Stable, bright in appearance.                               |
| 3           | 111                                                           | 10                        | 131                                  | 6                                 | 1                     | 133 Do.                                                         |
| 4           | 102                                                           | 7                         | 127                                  | 4                                 | 1                     | 129 Do.                                                         |
| 5           | 93                                                            | 1                         | 117                                  | -6                                | 2                     | 130 119 Do.                                                     |
| 6           | 111                                                           | 10                        | 128                                  | 5                                 | 1                     | 134 136 Do.                                                     |
| 7           | 91                                                            | 1                         | 119                                  | -4                                | 1                     | 117 116 Do.                                                     |
| 8           | 108                                                           | 9                         | 126                                  | 2                                 | 1                     | 133 135 Do.                                                     |
| 9           | 112                                                           | 10                        | 130                                  | 7                                 | 1                     | 132 134 Do.                                                     |
| 10          | 107                                                           | 10                        | 129                                  | 7                                 | 1                     | 132 134 Do.                                                     |
| 11          | 108                                                           | 9                         | 129                                  | 7                                 | 1                     | 134 135 Do.                                                     |
| 12          | 111                                                           | 10                        | 133                                  | 8                                 | 1                     | 133 136 Do.                                                     |
| 13          | 90                                                            | 0                         | 116                                  | -7                                | 1                     | 117 117 Do.                                                     |
| 14          | 107                                                           | 10                        | 128                                  | 5                                 | 1                     | 133 136 Do.                                                     |
| 15          | 89                                                            | -1                        | 116                                  | -7                                | 1                     | 115 114 Do.                                                     |
| 16          | 112                                                           | 10                        | 129                                  | 7                                 | 1                     | 134 137 Do.                                                     |
| 17          | 111                                                           | 10                        | 129                                  | 8                                 | 1                     | 133 136 Do.                                                     |
| 18          | 95                                                            | 3                         | 115                                  | -7                                | 5                     | 121 119 Phase separation, precipitation of optical brightener.  |
| 19          | 111                                                           | 10                        | 127                                  | 5                                 | 1                     | 134 134 Stable, bright in appearance.                           |
| 20          | 111                                                           | 9                         | 133                                  | 9                                 | 1                     | 134 137 Do.                                                     |
| 21          | 89                                                            | 0                         | 115                                  | -8                                | 5                     | 115 Phase separation, precipitation of optical brighteners.     |
| 22          | 91                                                            | 1                         | 116                                  | -7                                | 2                     | 111 110 Do.                                                     |
| 23          | 92                                                            | 2                         | 118                                  | -4                                | 5                     | 117 118 Do.                                                     |
| 24          | 89                                                            | 1                         | 114                                  | -8                                | 3                     | 121 121 Do.                                                     |
| 25          | 90                                                            | 1                         | 109                                  | -4                                | 4                     | 112 112 Do.                                                     |
| 26          | 93                                                            | 2                         | 109                                  | -4                                | 3                     | 120 120 Do.                                                     |
| 27          | 92                                                            | 0                         | 107                                  | -6                                | 5                     | 109 110 Stable, bright in appearance.                           |
| 28          | 94                                                            | 2                         | 109                                  | -4                                | 5                     | 110 112 Do.                                                     |
| 29          | 91                                                            | 0                         | 119                                  | -3                                | 3                     | 121 122 Phase separation, precipitation of optical brighteners. |
| 30          | 92                                                            | 0                         | 112                                  | -1                                | 3                     | 110 111 Stable, bright in appearance.                           |
| Blank       | 89                                                            | 0                         | 124                                  | 0                                 | 125                   | 123                                                             |

The following remarks are made on the results shown in Table 1. First, the basis of the interpretation of the data is follows: The reflectance of the swatch not treated with optical brightener is 89 at  $\lambda_{\text{max}} 440 \text{ m}\mu$  and, therefore, values over 89% prove whitening effects. The reflectance of the swatch treated with optical brightener (Whitex BB conc.) is 124 and, therefore, the swatches under 124 prove that they are quenched or yellowed by the cationic softening agent. On the other hand, the swatches over 124 prove that they are whitened by the fabric softener.

The same standard of evaluation will apply to the values of the swatches treated 5 and 10 times in the Test 2.

Now, the remarks are as follows:

(1) The formulations 1 to 8 are examples in which the third ingredient is a compound to be represented by a general formula similar to the above Formula VI. Because there is no  $-(\text{CH}_2\text{CH}_2\text{O})_n\text{H}$  chain in the third ingredient used in the formulation 1, it is an unstable composition. Accordingly, no whitening effect and no prevention of yellowing are recognized with respect to the formulation 1, and tinting phenomena are remarkable. The formulations 2, 3, 4, 6 and 8 relate to the ones in which the third ingredient belonging to the present invention is incorporated. The formulation 4 shows that the effect is smaller because the mole number of ethylene oxide is 14. The formulations 5 and 7 show that, when  $n$  of the  $-(\text{CH}_2\text{CH}_2\text{O})_n\text{H}$  chain is more than 15, the substantivity of optical brighteners will be reduced, so that no whitening effect and no prevention of yellowing are obtained. The third ingredient having  $-(\text{CH}_2\text{CH}_2\text{O})_n\text{H}$  chain in which  $n$  is more

45

chain in which  $n$  is less than 15. The formulations 9 and 10 relate to examples having a kind of alkyl radical, respectively, the formulation 11 relates to an example having  $\text{R}_{17}\text{CONHCH}_2\text{CH}_2-$ , and the formulation 12 relates to an example having

50



It is remarked that the formulation 13 relates to an example having an alkyl radical and, when



of this type of the third ingredient is unreasonably long, the substantivity of optical brightener is inferior.

(3) The formulations 14 and 15 relate to examples having a compound of the general Formula VIII. The formulation 14 relates to an example having an ethylene oxide chain of 10 moles and the formulation 15 relates to an example having an ethylene oxide chain of 20 moles. It should be noted that the ethylene oxide chain connected by  $\text{R}_3$  is different from a chain having an hydroxy group on the end of the chain. This means that  $\text{X}$  and  $\text{Y}$  of the compound of the general Formula VIII must be  $\text{X}+\text{Y} \leq 14$ .

(4) The formulations 16 to 18 relate to examples having a compound of the general Formula IX. The formulations 16 and 17 relate to examples having a third ingredient belonging to the present invention, respectively, and the formulation 18 relates to an example having no  $-(\text{CH}_2\text{CH}_2\text{O})_n\text{H}$  chain and it shows that the effects are inferior in such a case.

55

60

65

70

75

- (5) The formulation 19 in Table 1 relates to an example having a compound of the general Formula X, and it shows that all of the effects are excellent.
- (6) The formulations 20 and 21 relate to examples having compounds of the general Formula XI. The formulation 20 is excellent, but the formulation 21 shows that any remarkable effect is not obtained because of the presence of no  $-(CH_2CH_2O)_nH$  chain. 5
- (7) The formulation 22 in Table 1 shows that it does not have an effect of improving the substantivity of the optical brightener, because it contains a non-ionic surface active agent. 10
- (8) The formulation 23 shows that, when only a cationic surface active agent of the general Formula I and an optical brightener of the general Formula V are blended, a precipitation occurs, so that there is no adsorption of the optical brightener on the fabrics. 15
- (9) The formulations 24 to 26 shows that, even though a cationic surface active agent of the general Formula I is formulated with the third ingredient belonging to 20
- (10) The formulations 27 and 28 show that the formulation in the combination of a cationic active agent of the general Formula I, the third ingredient of the present 25 invention and a cationic optical brightener of the general Formula III or IV, but it never adsorbs on cellulose textiles and there is no whitening effect.
- (11) The formulation 29 shows that, when the optical 30 brightener is that of the general Formula II and the third ingredient is a non-ionic surface active agent the composition has no action of stabilizing a complex of the optical brightener with a cationic surface active agent in the system, and the optical brightener does not adsorb on the fabrics. The formulation 30 shows that, when the optical brightener is that of the general 35 Formula III and the third ingredient is a non-ionic surface active agent, the formulation is stable, but the optical brightener slightly adsorbs on fabrics.
- What we claim is: 40

1. A textile treating composition consisting essentially of:

- (1) 1 to 10 parts by weight of cationic surface active agent of the formula 45



wherein  $R_1$  and  $R_2$  are alkyls having 12 to 22 carbon atoms,  $R_3$  and  $R_4$  are alkyls having 1 to 4 carbon atoms, and  $X$  is halogen,  $CH_3SO_4^-$  or  $C_2H_5SO_4^-$  50

- (2) 0.05 to 0.5 part by weight of optical brightener of the formula 55



wherein  $M$  is alkali metal or ethanolamine, and 60

- (3) 0.5 to 10 parts by weight of cationic surface active agent selected from the group consisting of

(a) a compound of the formula



wherein  $R_{11}$  and  $R_{12}$  are  $-CH_3$ ,  $-C_2H_5$ , 70



$-CH_2R_{15}$ ,  $-(CH_2)_kNHCOR_{15}$  or  
 $-(CH_2)_kOOCR_{15}$

(wherein  $R_{15}$  is alkyl having 11 to 21 carbon atoms and  $k$  is an integer of from 1 to 3) and either one of  $R_{11}$  or  $R_{12}$  is  $-CH_2R_{15}$ ,



or  $-(CH_2)_kOOCR_{15}$ ;  $R_{13}$  is  $-CH_3$ ,  $-C_2H_5$ ,  
 $-CH_2-$

or  $-(CH_2CH_2O)_mH$ ,  $R_{14}$  is  $-(CH_2CH_2O)_nH$ ,  $m$  and  $n$  are integers of more than one, and  $2 \leq m+n \leq 14$ ,  $X_1^-$  is halogen,  $CH_3SO_4^-$  or  $C_2H_5SO_4^-$ ;

(b) a compound of the formula



wherein  $R_{21}$  is  $-CH_2R_{26}$ ,  $-(CH_2)_kNHCOR_{26}$  or  $-(CH_2)_kOOCR_{26}$ , (wherein  $R_{26}$  is alkyl having 11 to 21 carbon atoms and  $k$  is an integer from 1 to ),  $R_{22}$ ,  $R_{23}$  and  $R_{24}$  each is



$-(CH_2CH_2O)_mH$  or  $-(CH_2CH_2O)_nH$ , and  $l$ ,  $m$  and  $n$  each is an integer of more than one, and  $3 \leq l+m+n \leq 14$ ,  $R_{25}$  is  $-CH_3$ ,  $-C_2H_5$  or



$X_2^-$  and  $Y_2^-$  are halogen,  $CH_3SO_4^-$  or  $C_2H_5SO_4^-$ ;  $i$  is an integer of from 2 to 3;

(c) a compound of the formula



wherein  $R_{31}$  and  $R_{32}$  are alkyls having 12 to 21 carbon atoms,  $R_{33}$  is alkylene having more than 2 carbon atoms,  $R_{34}$  is  $-CH_3$ ,  $-C_2H_5$  or



$m$  and  $n$  are integers of more than one, and  $2 \leq m+n \leq 14$ ,  $x$  and  $y$  are integers of more than one, and  $2 \leq x+y \leq 14$ , and  $X_3^-$  and  $Y_3^-$  are halogen,  $CH_3SO_4^-$  or  $C_2H_5CO_4^-$ ;

(d) a compound of the formula



wherein  $M$  is



$R_{40}$  is alkyl having 12 to 21 carbon atoms,  $s$  is 2 or 3,  $p$  and  $q$  are integers of more than one, and  $2 \leq p+q \leq 14$ , and  $X_4^-$  is an anion obtained by removing one hydrogen from acetic acid, lactic acid, hydroxyacetic acid, boric acid or benzoic acid;

(e) a compound of the formula



wherein  $R_{50}$  is alkyl having 11 to 21 carbon atoms,  $R_{51}$  is  $-CH_3$ ,  $-C_2H_5$  or



**15**

*t* is an integer from 1 to 14, and  $X_5^-$  is halogen,  $CH_3SO_4^-$  or  $C_2H_5SO_4^-$ ;  
(f) a compound of the formula



wherein  $R_{60}$  is alkyl having 11 to 21 carbon atoms.

**16**

|             |         |               |       |           |
|-------------|---------|---------------|-------|-----------|
| 2,773,068   | 12/1956 | Mannheimer    | ----- | 252—542 X |
| 3,382,200   | 5/1968  | Buell         | ----- | 252—8.75  |
| 3,537,993   | 11/1970 | Coward et al. | ----- | 252—8.75  |
| 3,546,115   | 12/1970 | Gill et al.   | ----- | 252—8.8   |
| 5 3,630,895 | 12/1971 | Krause et al. | ----- | 252—8.75  |

## FOREIGN PATENTS

1,583,595 10/1969 France.

10 HERBERT B. GUYNN, Primary Examiner

U.S. CL. X.R.

## UNITED STATES PATENTS

|           |         |               |       |           |                                                     |
|-----------|---------|---------------|-------|-----------|-----------------------------------------------------|
| 2,304,369 | 12/1942 | Morgan et al. | ----- | 260—239   | 117—33.5 T, 139.5 C, O; 252—8.7, 8.8, 301.2 W; 260— |
| 2,933,529 | 4/1960  | Hwa           | ----- | 260—567.6 | 15 505 C                                            |

UNITED STATES PATENT OFFICE  
CERTIFICATE OF CORRECTION

Patent No. 3 781 204

Dated December 25, 1973

Inventor(s) Mamoru Katsumi, Toshio Sato and Tadao Hara

It is certified that error appears in the above-identified patent and that said Letters Patent are hereby corrected as shown below:

Col. 14, line 22; change "from 1 to )" to ---from 1 to 3)---.

Col. 14, line 32; change "C<sub>2</sub>H<sub>5</sub>SO<sub>4</sub>- i is" to ---C<sub>2</sub>H<sub>5</sub>SO<sub>4</sub>- , and  
i is---.

Col. 14, line 47; change "C<sub>2</sub>H<sub>5</sub>CO<sub>4</sub>" to ---C<sub>2</sub>H<sub>5</sub>SO<sub>4</sub>---.



Col. 14, line 56; change " -C-N-C-" to --- -C-N-C- ---.

Signed and sealed this 18th day of June 1974.

(SEAL)

Attest:

EDWARD M.FLETCHER, JR.  
Attesting Officer

C. MARSHALL DANN  
Commissioner of Patents